

## UNITED STATES PATENT OFFICE

2,537,106

## POLY-ACETOACETYL DERIVATIVES OF POLYAMINES AS AZO COMPONENTS IN DIAZOTYPE PHOTOPRINTING MATERIAL

William H. von Glahn, Loudonville, and Lester N. Stanley, Delmar, N. Y., assignors to General Aniline & Film Corporation, New York, N. Y., a corporation of Delaware

No Drawing. Application October 18, 1946,  
Serial No. 704,302

9 Claims. (Cl. 95—6)

1

This invention relates to a diazotype process and more particularly to the use of certain azo components in the light-sensitive layer of a diazotype reproduction medium or in a developing solution for the exposed diazotype image.

In the reproduction of mechanical drawings, printed material, pictures or other originals to be copied, it is of particular advantage in many cases to make first an intermediate print or transition print on a transparent diazotype copying material by exposing the transparent sensitized diazotype material to actinic rays such as ultraviolet light by either the printing through or reflex process and then developing the diazotype material. The development of such diazotype prints may be carried out by any of the developing methods known to the art for development of exposed diazotype materials. Thus, where a two-component system is employed containing the azo component in the light-sensitive layer with the diazo compound, development is effected by passing the exposed diazotype through ammonia vapors, and where a one-component system is employed which contains the diazo compound as the only dye component in the light-sensitive layer, the image is developed by treating the exposed diazotype with an alkaline solution containing the azo component by a dipping or fog spraying method. The image thus produced on the transparent intermediate or transition diazotype print can be used for reproduction of further diazotype prints of high contrast. If desired, they can also be used for the reproduction of the image on any suitable photoprinting material such as silver halide photographic paper and Van Dyke prints and blueprints.

This method of producing transition diazotype prints is particularly useful when it is desired to make a number of reproductions from a frail or valuable original which would be adversely affected if not destroyed in the repeated exposures necessary to make the desired number of copies. It is essential in the so-called reflex process where the diazotype copy material is superimposed on the opaque original to be copied and the light for exposure of the diazotype material passes through it and is reflected by the surface of the original. The efficiency of the process involving the production of a transition or intermediate print depends upon the opacity of the azo dye image produced upon such intermediate or transition print to ultraviolet light and upon the transparency of the background to such light. It depends also upon the visual density of

2

the image produced on the intermediate or transition print since images of poor visual density such as light yellows on a white or transparent background, though they may have the desired degree of opacity to ultraviolet light nevertheless have the disadvantage of rendering difficult the detection of flaws in the intermediate image. With such prints, it is necessary to make a contrast print of good visual density from the intermediate before such flaws can be detected thereby introducing an additional and unnecessary step.

Prints of a deep color having good visual density can be obtained from diazotypes using azo components common to the art for the production of ordinary diazotypes such as phloroglucin, 2,3-dihydroxynaphthalene and  $\beta$ -naphthol-3,6-disulfonic acid. However, despite the good visual density of the color reproducing the image, its actinic opacity or photographic density is not sufficient to reproduce the image satisfactorily in subsequent copies. The azo dye component used for the production of transition print images must be such as to produce upon coupling with the diazo compound employed a color which will sufficiently absorb the ultraviolet light incident upon it during exposure to prevent light-decomposition of the diazo compound in the areas to be reproduced from the transition copies. Colors of good visual density do not necessarily have this property. It is well known for instance that blues such as are produced from azo components like phloroglucin are very poor in their ultraviolet absorption characteristics.

Azo components such as resorcinol have heretofore been employed in the production of diazotype prints in order to obtain color images having the necessary light absorption characteristics for transition printing. Resorcinol will reproduce the image on the transition print in a sepia or orange-brown color which has good opacity to ultraviolet light and has sufficient depth of color or visual density to assure detection of printing flaws and the like in the developed intermediate print. Other azo components have been suggested which will produce images of good opacity or covering power when used in combination with poly hydroxy azo components such as phloroglucinol and resorcinol. These azo components are acetoacetyl derivatives of monoamines and are disclosed in Patent #1,989,065. However, although these acetoacetyl derivatives of mono-amines may produce satisfactory results as shaders for other colors which may lack the necessary covering power, particularly in copying half tones or too light lines, they do not produce

satisfactory images when used as self colors, that is, when the acetoacetyl derivatives of monoamines such as the cyclohexyl acetoacetic acid amide and the like disclosed in Patent #1,989,065 are used as the only azo components for the development of a diazotype print, the image produced does not have a satisfactory shade or tone value.

It has now been found that the polyacetoacetyl derivatives of aliphatic, aromatic or heterocyclic polyamines are especially effective as azo components or diazotype reproductions. This class of azo components can be used satisfactorily either alone in the production of self shades or in combination with other azo components for shading purposes. In either case the resulting images have excellent opacity characteristics. The opacity to ultraviolet light and covering power of the self shades markedly surpass those properties of colors produced from the monoacetoacetyl derivatives and when used for shading purposes in combination with such azo components as phloroglucinol, 2,3-dihydroxy naphthalene or 2,3-dihydroxy naphthalene sulfonic acid, excellent neutral blacks having good opacity to ultraviolet light are obtained. In general these polyacetoacetyl derivatives are prepared from the corresponding polyamine by reaction with acetoacetic esters or with diketenes. The acetoacetic ester or diketene condenses with the amino groups of the polyamine thus forming amide linkages. The amine may be any aliphatic, aromatic or heterocyclic polyamine wherein the aliphatic chain or aromatic or heterocyclic nuclei may be substituted by any of the usual substituents such as alkyl, halogen, alkoxy, carboxy, sulfo, hydroxy or other groups which do not discolor the paper or impair the solubility characteristics of the azo component. (For example, nitro groups discolor the paper.) This class of azo components may be represented by the following general formula:  $R(COCH_2COCH_3)_n$  wherein R is an aliphatic aromatic or heterocyclic polyamino radical and n is a whole number greater than one and each acetoacetyl group is attached to an amino nitrogen atom of R. Examples of polyacetoacetyl derivatives of this class are:

1. N-( $\beta$ -acetoacetaminoethyl)-acetoacetamide



2. N-( $\beta$ -acetoacetaminopropyl)-acetoacetamide



3. N,N'-(acetoacetylmino-diethylene)-diacetoacetamide



4. 2,4-diacetoacetamino-benzene sulfonic acid



5. 2,4-diacetoacetamino-toluene



6. Bis-acetoacet-o- or m-dianiside



7. Diacetoacetyl-piperazine



8. N(N'-diacetoacetyl-4-amino piperidine



9. Triacetoacetyl-melamine



10. Diacetoacetyl-benzidine



11. 1,4-diacetoacetamino-naphthalene



In the preparation of diazotype materials intended for use as intermediate or transition print media in accordance with this invention, a suitable transparent base such as transparentized paper, cellulose acetate film or other transparent material is coated by means known to the art with a light-sensitive composition containing suitable diazo compounds. Where it is desired to make a two-component diazotype layer on the support or base material for development by the dry developing method, the azo component is also incorporated into the coating composition. Where one-component diazotype layers are desired, the azo component is added to an alkaline developing solution and after exposure of the diazotype the exposed image is developed by contacting with the alkaline developing solution by means known to the art. In the preparation of coating compositions for two-component diazotype layers, the coating solution may also contain such other materials as are ordinarily used in the preparation of diazotype two-component light-sensitive coating compositions. These include stabilizing materials such as citric acid, phosphoric acid and thiourea; swelling agents for cellulose acetate and other cellulosic ester bases such as isopropanol, and shade intensifying agents, such as nickel sulfate. In the preparation of light-sensitive layers on paper for the production of neutral black images or dark tone images which may or may not be intended for reproduction of further copies, it is preferable to employ a two-component coating composition which will contain

one or more dark tone producing azo components, preferably such as will produce blue shades with the diazo compounds employed in combination with the polyacetoacetyl amino azo components of this invention. The diazo compound or compounds and other adjuvants are added to the coating composition and the paper used as a carrier for the light-sensitive layer is coated in the same manner as the transparentized paper or cellulose film base material in the case of the transition print media. As diazo compounds any suitable light-sensitive diazo compound which will couple with the azo components to reproduce a colored image may be employed. We prefer, however, to use diazo compounds derived from p-diamines of the benzene series, particularly when two-component coating compositions are employed. As is well known in the art, this class of diazo compounds is especially suitable for the production of two-component diazotype photo-sensitized papers. Other diazo compounds have been found suitable for use such as diazo anhydrides of aminohydroxynaphthalene compounds but are less extensively employed. The p-diamines most generally used for production of the diazo compounds are those wherein one of the amino groups is unsubstituted for diazotization and the other is substituted by such groups as alkyl, alkoxy-alkyl, aryl, aralkyl, alkylol, cycloaliphatic and heterocyclic groups. Examples of these amines from which the diazo compounds are derived include N-hydroxyethyl-N-methylamino-p-aminobenzene; p-amino-diphenylamine; 1-mono-methylamino-2(or 3)-methyl-4-aminobenzene; 1-N-hydroxyethyl-N-ethylamino-3-methyl-4-aminobenzene; 1-diethylamino-3-ethoxy-4-aminobenzene; 4-amino-1-benzoylamino-2,5-diethoxybenzene; p-amino-N-diethylaniline; 1-N,N-dihydroxyethylamino-3-chloro-4-aminobenzene; p-amino-N-ethyl-N-benzylaniline; 1-ethyl-4-aminobenzene; 1-N-hydroxyethyl-N-ethylamino-4-aminobenzene; p-phenylene diamine; 4-amino-N,N-dihydroxyethylaniline; p-(4'-ethoxy phenyl)amino-2,5-diethoxyaniline; 1-N-ethylamino-2-methyl-4-aminobenzene; 1-dimethylamino-3-methoxy-4-aminobenzene; N,N-dimethylamino-p-aminobenzene; 1-dimethylamino-3-methyl-4-aminobenzene; p-aminophenyl morpholine and 2-amino-1-naphthol-5-sulfonic acid. The diazo derivatives of these amines are used in the form of their stabilized salts, such as the ZnCl<sub>2</sub>, CdCl<sub>2</sub> or SnCl<sub>2</sub> double salts, fluoro borates, aryl or alkyl sulfonates, and acid sulfates of the diazonium chloride.

The following specific examples will serve to illustrate further the invention, it being understood, however, that they are not intended to limit its scope. Unless otherwise stated, the parts are by weight.

#### Example I

Transparentized paper is coated with a coating solution containing the following materials per 100 cc. of a 5% aqueous solution of alcohol:

3.5 g. N-( $\beta$ -acetoacetaminoethyl)-acetoacetamide  
3.8 g. N-methyl, N-hydroxyethylamino-p-benzene diazonium chloride-ZnCl<sub>2</sub> double salt  
4.0 g. thiourea  
8.0 g. citric acid  
2.0 g. phosphoric acid  
5.0 g. zinc chloride

The coated transparency is first dried in the usual manner. It is then exposed to actinic light under a pattern and developed by contacting with

ammonia fumes. The image of the pattern is developed in an orange sepia shade against a clear background of the transparentized paper base. This print has excellent qualities of opacity to ultraviolet light in the dye areas and is, therefore, eminently suited to further reproduction work. The dye image of this transparency is also highly resistant to fading so that a large number of reproductions can be made from it and it has good wash-fastness properties.

#### Example II

Transparentized paper is coated with a coating solution containing the following ingredients per 100 cc. of a 5% aqueous solution of alcohol:

3.5 g. N-( $\beta$ -acetoacetaminoethyl)-acetoacetamide  
3.5 g. N,N-diethylamino-p-benzene diazonium chloride-ZnCl<sub>2</sub> double salt  
4.0 g. thiourea  
8.0 g. citric acid  
2.0 g. phosphoric acid  
5.0 g. zinc chloride

The coated transparency is first dried in the usual manner and is then exposed to light under a pattern and developed by contacting with ammonia fumes. The image of the pattern is developed in a deep orange sepia shade which possesses excellent opacity to ultraviolet light. It is therefore well suited for further reproduction work as a transition print. Its light-fastness and wash-fastness properties are similar to the prints obtained in accordance with Example I.

#### Example III

Transparentized paper is coated with a coating solution containing the following ingredients per 100 cc. of a 5% aqueous solution of alcohol:

3.5 g. N-( $\beta$ -acetoacetaminoethyl)-acetoacetamide  
3.6 g. 1-N-ethylamino, 2-methyl-4-benzene diazonium chloride-ZnCl<sub>2</sub> double salt  
4.0 g. thiourea  
8.0 g. citric acid  
2.0 g. phosphoric acid  
5.0 g. zinc chloride

The coated transparency is first dried in the usual manner and is then exposed to light under a pattern and developed by contacting with ammonia fumes. The image of the pattern is reproduced in an orange-yellow shade having excellent opacity to ultraviolet light. The light-fastness and wash-fastness properties of this print are also good and it is particularly suited for use as a transition print in the reproduction of further copies.

#### Example IV

Transparentized paper is coated with a coating solution containing the following ingredients per 100 cc. of a 5% aqueous solution of alcohol:

5.8 g. N-( $\beta$ -acetoacetaminopropyl)-acetoacetamide  
3.8 g. N-methyl, N-hydroxyethylamino-p-benzene diazonium chloride-ZnCl<sub>2</sub> double salt.  
4.0 g. thiourea  
8.0 g. citric acid  
2.0 g. phosphoric acid  
5.0 g. zinc chloride

The coated transparency is first dried in the usual manner and is then exposed under a pattern and developed by contacting with ammonia fumes. The image of the pattern is reproduced

in an orange-yellow print. This transition print possesses excellent opacity to ultraviolet light in the dye areas and is therefore particularly suited for further reproduction work. Its light-fastness and wash-fastness properties are also good.

Upon substituting 4.0 g. 1-(n-ethylamino)-2-methyl-4-benzene diazonium chloride-ZnCl<sub>2</sub> double salt or 4.5 g. N-ethyl, N-hydroxyethylamino-p-benzene diazonium chloride-ZnCl<sub>2</sub> double salt for the 3.8 g. N-methyl, N-hydroxyethylamino-p-benzene diazonium chloride-ZnCl<sub>2</sub> double salt of this example, orange-yellow prints of outstanding opacity characteristics having the same light-fastness and wash-fastness properties as the prints of this example, may be obtained.

*Example V*

Transparentized paper is coated with a coating solution containing the following ingredients per 100 cc. of a 5% aqueous solution of alcohol:

2.3 g. N,N'-(acetoacetylaminodiethylene)-diacetacetamide  
3.8 g. N-methyl, N-hydroxyethylamino-p-benzene diazonium chloride-ZnCl<sub>2</sub> double salt  
4.0 g. thiourea  
8.0 g. citric acid  
2.0 g. phosphoric acid  
5.0 g. zinc chloride

The coated transparency is first dried in the usual manner. It is then exposed to light under a pattern and developed by contacting with ammonia fumes. Deep orange sepia colored prints are produced of very good covering power. These prints may be used as transition prints in the reproduction of further copies due to their high opacity to ultraviolet light, light-fastness and wash-fastness properties. The azo component of this example may be used in even smaller amounts than indicated in this example while still obtaining deep shaded prints having good opacity to ultraviolet light.

Upon substituting 3.5 g. N-phenylamino-p-benzene diazonium acid sulfate for the 3.8 g. N-methyl, N-hydroxyethylamino-p-benzene diazonium chloride-ZnCl<sub>2</sub> double salt of this example, brown prints having excellent opacity characteristics are obtained.

*Example VI*

Transparentized paper is coated with a coating solution containing the following ingredients per 100 cc. in a 5% aqueous solution of alcohol:

7.0 g. 2,4-diacetoacetamino-benzene sulfonic acid  
3.8 g. N-methyl, N-hydroxyethylamino-p-benzene diazonium chloride-ZnCl<sub>2</sub> double salt  
4.0 g. thiourea  
8.0 g. citric acid  
2.0 g. phosphoric acid  
5.0 g. zinc chloride

The coated transparency is first dried in the usual manner. It is then exposed to light under a pattern and developed by contacting with ammonia fumes. Sepia prints of the pattern are thus obtained having good opacity to ultraviolet light, excellent light-fastness and wash-fastness properties. These prints are eminently suited for use in transition prints in the reproduction of further copies.

By replacing the diazo compound of this example with 4.5 g. N,N-dimethylamino-p-benzene diazonium chloride-ZnCl<sub>2</sub> double salt, similar sepia prints having the same good opacity, light-fastness and wash-fastness properties are obtained.

*Example VII*

Transparentized paper is coated with a 5% solution of 1-benzoylamino-2,5-diethoxy-4-benzene diazonium chloride-ZnCl<sub>2</sub> double salt in 100 cc. of water containing 5% alcohol, 4% thiourea and 0.5% saponin.

The coated transparency is first dried in the usual manner and then exposed to light under a pattern. The print is developed moist by applying a 5% solution of (N-( $\beta$ -acetoacetaminoethyl)-acetoacetamide containing 5 g. of Na<sub>2</sub>CO<sub>3</sub> per 100 cc. of solution.

The sepia print of the pattern thus obtained has outstanding opacity characteristics. It also has good light-fastness and wash-fastness properties.

*Example VIII*

Ordinary paper stock for diazotypes is coated 20 with a coating solution containing the following ingredients per 100 cc. of a 3% aqueous solution of isopropanol:

1.4 g. N-( $\beta$ -acetoacetaminoethyl)-acetoacetamide  
25 3.0 g. 2,3-dihydroxynaphthalene-6-sulfonic acid  
0.15 g. 2,5-dihydroxynaphthalene  
3.0 g. N,N-diethylamino-p-benzene diazonium chloride-ZnCl<sub>2</sub> double salt  
30 5.0 g. ZnCl<sub>2</sub>  
10.0 g. citric acid  
2.0 g. phosphoric acid  
5.0 g. thiourea

The coated paper is first dried in the usual manner and is then exposed under a pattern and developed by contacting with ammonia fumes. The prints thus developed are a neutral black shade having good gradation and showing little tendency for color shift upon standing. These prints also have good opacity to ultraviolet light and good light-fastness and wash-fastness properties.

Upon substituting the following mixtures of azo components for the three azo components in the formula of this example, diazotype prints 45 having similar characteristics and properties are obtained:

(1) 1.0 g. 2,4-diacetoacetamino-toluene  
3.0 g. 2,3-dihydroxynaphthalene-6-sulfonic acid  
50 0.12 g. 2,3-dihydroxynaphthalene  
(2) 1.0 g. bis-acetoacet-o-dianisidine  
2.8 g. 2,3-dihydroxynaphthalene-6-sulfonic acid  
55 0.1 g. 2,3-dihydroxynaphthalene

The coating, formula and procedure are otherwise the same as in this example. The compositions of this example illustrate the utility of the polyacetoacetyl polyamines of this invention for shading to neutral blacks when they are used in mixture with azo components which normally develop to a blue shade. Other azo components which will develop blue shades, such as phloroglucinol, may be substituted for or combined with the 2,3-dihydroxynaphthalene couplers of this example with similar results and azo components which will produce tones other than blue may also be used in combination with the polyacetoacetyl polyamines to produce modified tones which will have good covering power and opacity to ultraviolet light.

We claim:

1. A diazotype photoprinting material comprising a light-sensitive diazo compound and an 75 azo component selected from the class consisting

of polyacetoacetyl derivatives of aliphatic polyamines wherein the acetoacetyl groups are attached to amino nitrogen atoms of the polyamines.

2. A diazotype photoprinting material comprising a light-sensitive diazo compound and an azo component selected from the class consisting of polyacetoacetyl derivatives of aliphatic polyamines wherein the acetoacetyl groups are attached to the nitrogen atoms of the polyamines and another azo component.

3. A diazotype photoprinting material comprising a light-sensitive diazo compound and as azo component the compound  $N-(\beta\text{-acetoacetoaminoethyl})\text{-acetoacetamide}$  having the structural formula:



4. A diazotype photoprinting material comprising a light-sensitive diazo derivative of a p-diamine of the benzene series and as azo component the compound  $N-(\beta\text{-acetoacetaminoethyl})\text{-acetoacetamide}$  having the structural formula:



5. A diazotype photoprinting material comprising a salt of  $N$ -diethylamino-p-benzene diazonium chloride and  $N-(\beta\text{-acetoacetaminoethyl})\text{-acetoacetamide}$  having the structural formula:



6. A diazotype photoprinting material comprising a salt of  $N,N$ -diethylamino-p-benzene diazonium chloride,  $N-(\beta\text{-acetoacetaminoethyl})\text{-acetoacetamide}$ , 2,3-dihydroxynaphthalene and 2,3-dihydroxynaphthalene-6-sulfonic acid.

7. A diazotype photoprinting material comprising a light-sensitive diazo compound and as azo component the compound  $N,N'$ -(acetoacetyl imino - diethylene) - diacetoacetamide, having the structural formula:



8. A diazotype photoprinting material comprising a light-sensitive diazo derivative of a p-diamine of the benzene series and as azo component the compound  $N,N'$ -(acetoacetyl imino - diethylene) - diacetoacetamide, having the structural formula:



9. A diazotype photoprinting material comprising a salt of  $N$ -methyl,  $N$ -hydroxyethylamino-p-benzene diazonium chloride and  $N,N'$ -(acetoacetyl imino - diethylene) - diacetoacetamide, having the structural formula:



WILLIAM H. VON GLAHN.  
LESTER N. STANLEY.

#### REFERENCES CITED

The following references are of record in the file of this patent:

#### UNITED STATES PATENTS

| Number    | Name        | Date          |
|-----------|-------------|---------------|
| 1,822,065 | Sprongerts  | Sept. 8, 1931 |
| 1,972,323 | Shiraeff    | Sept. 4, 1934 |
| 1,989,065 | Schmidt     | Jan. 22, 1935 |
| 2,010,884 | Olpin       | Aug. 13, 1935 |
| 2,027,229 | Hinman      | Jan. 7, 1936  |
| 2,250,129 | Kopp et al. | July 22, 1941 |
| 2,299,641 | Middleton   | Oct. 20, 1942 |
| 2,312,040 | Kendall     | Feb. 23, 1943 |
| 2,331,812 | Steiger     | Oct. 12, 1943 |
| 2,395,776 | Bavley      | Feb. 26, 1946 |

#### OTHER REFERENCES

Spencer: "Photographic Applications of Diazo Compounds," The Photographic Journal (London), December 1928, pages 490 to 496, page 494 cited (copy in S. L.).